

April 16, 1946.

W. J. MALCOLMSON ET AL

2,398,712

MANUFACTURE OF COATED ARTICLES

Filed Sept. 4, 1942

FIG. 1



FIG. 2

INVENTORS

W. J. MALCOLMSON  
R. V. MINER

BY Harry L. Swift  
ATTORNEY

## UNITED STATES PATENT OFFICE

2,398,712

## MANUFACTURE OF COATED ARTICLES

William J. Malcolmson, Riverside, and Robert V. Miner, Western Springs, Ill., assignors to Western Electric Company, Incorporated, New York, N. Y., a corporation of New York

Application September 4, 1942, Serial No. 457,324

8 Claims. (Cl. 204—38)

This invention relates to the manufacture of coated articles and more particularly to an article having an adherent coating of noble metal on its surface and to a method of making such an article.

It is sometimes desirable to provide an article with a coating which will be both corrosion resistant and conductive. Certain metals, such as gold, silver and platinum, have been used for this purpose.

An object of this invention is to provide an article having a noble metal coating and an effective and efficient method for producing such an article.

In accordance with one embodiment of this invention, an article made of aluminum is first anodized and then coated with a liquid organic gold compound. The coated article is then fired to decompose the compound and to leave a thin gold film on the coated area.

In accordance with another embodiment of this invention, an article may be provided with a coating of aluminum, the aluminum anodized and then coated with a liquid organic gold compound. The coated article is fired and the compound decomposes, leaving a thin gold film on the coated area.

Other objects and advantages of this invention will be apparent from the following detailed description taken in conjunction with the following drawing:

Fig. 1 shows an enlarged plan view of a transmitter electrode coated in accordance with one embodiment of this invention, and

Fig. 2 is a sectional view of the same taken along the line 2—2 of Fig. 1.

In certain types of electrical apparatus, such as communication equipment, cup shaped members are often employed to make electrical contact with other portions of the apparatus and, in many instances, satisfactory performance of the apparatus necessitates that these contact members receive transmitted current without appreciable loss or distortion. For example, in certain types of telephone transmitters, cup shaped electrodes are used to provide the necessary electrical connections with the carbon particles therein and satisfactory operation of the transmitter depends in large measure upon the contact efficiency of these electrodes. In order to provide the needed operating and service characteristics, it is often desirable to use gold or some other noble metal as a contact material on these electrodes and, due to the very high cost of these noble metals, it is desirable to apply a thin film

and to restrict their use to the portions of the electrode surface which are actually in contact with the carbon.

An organic gold compound suitable for coating in accordance with this invention may be prepared in several ways. An organic gold compound having the empirical formula  $C_{10}H_{16}SAuCl_3$  may be prepared by mixing a terpene with sulphur or an alkali polysulphide and then mixing the product with a gold chloride. Other salts of heavy metals may also be used instead of the gold chloride, according to the metal coating desired. The compound may be diluted to the desired viscosity with an essential oil, such, for example, as oil of lavender or rosemary oil. A suitable compound may also be prepared by heating an essential oil containing a saturated alcohol or ester, such as terpineol, with sulphur. This mixture is then purified by distillation at from 120° C. to 130° C. under 20 mm. pressure. The purified product is then caused to react with a 10% aqueous solution of gold chloride mixed with resinate of bismuth, rhodium and chromium. The product is then diluted to the desired viscosity with an essential oil.

In practicing this invention, an article such as a transmitter electrode 3, shown in Fig. 1, made of aluminum is anodized by electrolyzing it with a bath of sulphuric acid or by any other suitable aluminum anodizing method. This produces a finely porous surface 4 to which the coating to be subsequently applied adheres excellently. The area which it is desired to coat is then coated either by brushing or spraying with a quantity of gold compound, or other noble metal, prepared as described above, the thickness of the coating being determined largely by the viscosity of the compound. The coated article is then fired at a temperature sufficient to decompose the compound and leave a thin, adherent film 5 of noble metal as a coating on the anodized aluminum surface.

It has been found that with some organic gold compounds, such as diethylmonobromogold, the compound will decompose fairly rapidly at room temperatures. However, using a gold compound prepared by the reaction of sulphur on terpenes as described above, it has been found desirable to use temperatures between 300° C. and 600° C. to accelerate the rate of decomposition. However, temperatures up to the melting point of the aluminum may be used if desired, since gold, silver and platinum have melting points substantially higher than that of the aluminum.

In coating articles other than articles of aluminum, in order to obtain an adherent coating of gold, or other noble metal, it has been found desirable to provide the article with a coating of anodized aluminum prior to coating with the organic gold compound. In this way, any article may be provided with an adherent coating of gold or other noble metal.

While this invention has been described in connection with coating with gold, the method is equally applicable to coating with other noble metals such as platinum or silver, an organic compound of either being used as the coating material. While but two embodiments of this invention have been described, it will be understood that many changes and modifications may be made therein without departing from the spirit or scope of the present invention.

What is claimed is:

1. A method of producing an article having a coating of noble metal which comprises providing the article with a base coating of aluminum having an anodized surface, coating the article with an organic compound of a salt of a noble metal, and then heating the coated article to decompose the compound.

2. A method of producing an article of aluminum having a coating of noble metal thereon which comprises anodizing the surface of the article, coating the article with an organic compound of a salt of a noble metal, and then heating the coated article to decompose the compound.

3. In a method of producing an article of aluminum having a coating of noble metal thereon which comprises anodizing the surface of the article, coating the article with an organic compound of a salt of a noble metal, and then heat-

ing the article to between 300° C. and 600° C. to decompose the compound.

4. A method of producing an article of aluminum having a coating of noble metal thereon comprising anodizing the surface of the article, coating the article with an organic gold salt compound, and then heating the coated article to decompose the compound.

5. A method of producing an article of aluminum having a coating of noble metal thereon comprising anodizing the surface of the article, coating the article with an organic gold compound, and then heating the article to between 300° C. to 600° C. to decompose the compound.

6. A method of producing an article of aluminum having a coating of noble metal thereon, comprising anodizing the surface of the article, coating the article with a solution of diethyl-monobromogold, and then decomposing the compound by the application of heat to leave a gold coating.

7. A method of producing an article having an aluminum surface with a coating of a noble metal which comprises anodizing the aluminum surface, applying an organic compound of a salt of said metal to the anodized surface, and decomposing said compound by the application of heat to leave a coating of said metal on said surface.

8. A method of obtaining a thin adherent film of gold on an article comprising providing the article with a surface of anodized aluminum, coating the article with an organic gold compound having the empirical formula  $C_{10}H_{16}SAuCl_3$ , and then heating the coated article to decompose the compound.

WILLIAM J. MALCOLMSON.  
ROBERT V. MINER.